

## UNITED STATES PATENT OFFICE

HARRY S. SCHUTTE, OF PITTSBURGH, PENNSYLVANIA

## TREATING FERROUS SHEETS AND PLATES

No Drawing.

Application filed July 31, 1930. Serial No. 472,186.

This invention relates to the manufacture of rolled sheets and plates such as tin plate and similar ferrous metal materials which, after being rolled, are pickled and then washed, and after being formed into a pile are later subjected to a box annealing operation preparatory to further finishing operations.

A most tedious and troublesome operation 10 in the manufacture of such materials, and particularly tin plate, has been the separation of the hot rolled sheets or plates in an annealed pile after the first box annealing operation. This separation, known as "opening", is essential because the pile of sheets or 15 plates have become welded together or adherent in varying degrees while undergoing the heat treatment to which the piles are subjected in such annealing operations. And the 20 same difficulties are encountered but to a lesser extent in box annealing cold rolled materials.

After the annealing operation it is necessary for each sheet to be freed from any temporary union with the others of the pile so 25 as to be ready for subsequent processing or use. While all of the sheets or plates in an annealing charge are not usually stuck together in the manner indicated, such condition is present to a very considerable extent 30 in practically every annealed pile of hot rolled material and to a degree in annealed piles of cold rolled materials. The result is that the slow, laborious and costly process of manually opening a pile of annealed materials has heretofore been a regular and un- 35 escapable feature of the mill routine.

The primary object of this invention is the provision of improved means whereby the objectionable welding or sticking together of 40 the sheets and plates ordinarily present after the box annealing operation is prevented or, to a large extent, overcome, and the labor necessary in opening the materials in readiness 45 for cold rolling and further treatment is reduced to a minimum; likewise, the reduction in and prevention of rust formation and substantial elimination of the destructive staining 50 of the surfaces of the sheets or plates generally present in the methods used hereto-

fore, are effected in a simple, rapid and economical manner.

Still further objects of the invention will be made apparent hereinafter in the detailed description and appended claims.

In the practice of the improved method the sheets or plates, after the removal of the scale and prior to annealing, are treated by dipping them in a suitable aqueous mixture or chemical solution, preferably a solution of sodium bichromate or sodium chromate.

With existing tin mill equipment it is possible to provide for the bichromate treatment by adding the chemical in proper proportions to the rinse or wash tank at the pickler. A concentration of 0.05 per cent. sodium bichromate or of sodium chromate in the wash water has been found sufficient to accomplish the desired results. Thus, the sheets or plates, as soon as the oxid or scale has been removed by the action of the pickling operation, are immersed, rinsed and treated in a dilute solution of sodium bichromate or sodium chromate, after which they are inspected in the usual manner and arranged in piles for the black annealing operation.

A more economical and effective method is to provide an additional dipping tank in which the sheets or plates to be treated are immersed in the solution or aqueous mixture after having been rinsed with water in the wash tank.

Whatever portion of the solution or mixture adheres to the sheets or plates as they are formed into piles on the charging stands is usually allowed to remain on the surfaces.

It has been found that this treatment practically eliminates troublesome sticking or welding of the sheets or plates in the subsequent annealing process; that better annealing is obtained; that the annealing temperature can be raised at least 100 degrees Fahrenheit; that the opening operation is greatly facilitated and that the spoilage of many sheets or plates in the opening operation is avoided. A reduction of approximately 50 per cent. in the cost of opening is thus effected.

Another apparent advantage of the bichromate or analogous treatment is a mate-

rial reduction in the amount of destructive staining on the surfaces of the materials which heretofore has contributed to the production of defective tin coatings.

5 The action of rust on the pickled materials while still wet apparently is retarded and in this way contributes to a better surface condition.

10 The term aqueous mixture as used herein is intended to cover any of the chemical solutions or mixtures specified as usable in practicing my invention.

15 While sodium bichromate is the best material found so far in accomplishing the results described above I have found that other materials likewise have beneficial effects. Other chromates and bichromates may be used. Potassium bichromate, of course, will give similar results, having properties similar 20 to those of sodium bichromate. The broad idea underlying this invention is in that the presence of a separating or reacting medium, extremely thin, and particularly a substance which in itself would militate against physical welding or sticking of the rolled material, will be beneficial.

25 While the fundamental concept lies in the use of a separating medium between sheets in a box annealing operation one important 30 feature was to find the materials of greatest efficiency which, at the same time, would not by their presence interfere with subsequent operations. Various chemical salts, oxidizing agents and compounds have been used to 35 good effect in the place of bichromate; for example, the chromates and among others are zinc sulphate, sodium permanganate, zinc chloride and/or zinc oxide, all of which have desirable properties in relation to this process.

40 In designating a concentration of 0.05 per cent. sodium bichromate as satisfactory I have given this figure only as being representative of the approximate minimum desirable in one particular embodiment of the 45 invention.

50 Higher concentrations may be maintained and the manner of application of the solution may be modified so that it will fit into any procedure for the production of rolled ferrous metal plates and the like. Concentrations as low as 0.001 per cent. have been 55 found to give beneficial results.

55 The advantages of my invention will be apparent to those skilled in the art. The materials used in forming the aqueous mixture with which the sheets and plates are treated are not limited to those specifically mentioned herein and other changes may be 60 made within the scope of the invention, as defined by the claims.

I claim:

65 1. The method of preventing sticking in box annealing sheets and plates which consists in chemically treating the rolled and pickled sheets and plates by immersion in an

aqueous solution of sodium bichromate of a concentration of .05 per cent., piling the treated materials and then box annealing the pile.

70 2. The method of preventing sticking in box annealing sheets and plates which consists in chemically treating the rolled and pickled sheets and plates by immersion in an aqueous solution of sodium bichromate of a concentration of .03 to .05 per cent., piling the 75 treated materials and then box annealing the pile.

80 3. The method of preventing sticking in box annealing sheets and plates which consists in chemically treating the rolled and pickled sheets or plates by immersion in an aqueous solution of a sodium salt of a chromic acid of a concentration of .001 to .20 per cent., piling the treated materials and then 85 box annealing the pile.

90 4. The method of preventing sticking in box annealing sheets and plates which consists in chemically treating the rolled and pickled sheets and plates by immersion in an aqueous solution of a salt of a chromic acid of a concentration of .001 to .20 per cent., piling the treated materials and then 95 box annealing the pile.

100 In testimony whereof, I have hereunto set my hand.

95 HARRY S. SCHUTTE.

100

105

110

115

120

125

130